

## UNITED STATES PATENT OFFICE

2,216,968

## METHOD FOR REFINING LUBRICATING OIL DISTILLATES

Hans G. Vesterdal, Elizabeth, N. J., assignor to  
Standard Oil Development Company, a corpora-  
tion of Delaware

No Drawing. Application May 28, 1938,  
Serial No. 210,749

6 Claims. (Cl. 196—41)

The present invention relates to an improved method for refining heavy hydrocarbon oils, especially of the type obtained from naphthenic crudes, which are susceptible to loss of color on standing or which contain impurities such as soaps having high ash contents. The invention will be fully understood from the following description.

Lubricating oil distillates are frequently susceptible to loss in color on standing. This appears to be a marked characteristic of the products derived from naphthenic base crudes such as are obtained from Colombia and the Coastal regions of the United States. These oils are largely used for making low cold test lubricants for industrial purposes. The cause of the loss of color is not fully understood, but it is believed to be due to the presence of small amounts of naphthenic acids and frequently to the presence of complex phenolic materials. It is now customary to refine these oils by treatment with acid but in order to obtain color stable oils according to this method, large amounts of sulfuric acid are required in the treatment and the treating loss is quite large. Residual oil containing soaps and having high ash content are also troublesome to handle by present methods, which give satisfactory products only at the cost of a considerable loss of oil.

It has been found that oils of these types can be readily refined without any acid treatment whatever and they are satisfactory for most of the purposes to which they are now put. If better oils are required, a limited acid treatment or solvent extraction treatment or other refining method may be used such as limited oxidation which are followed, if desired, with either acid or solvent refining. These various refining methods are used prior to the present finishing process but for most purposes this is not required. In the present process, the oil, whether a crude or a distillate or residue obtained by pipe still distillation or residue obtained in distillation over caustic soda, is treated under high temperature with say 10 to 500% of its volume of a dilute aqueous caustic alkali, preferably sodium hydroxide. The concentration of the alkali may be from 25 to 5% depending to some extent on the character of the oil to be refined, its viscosity, and the amount of impurity to be removed. It is preferred to use solutions in the more dilute portion of the range specified hereinabove, and the volume used is preferably 10 to 100% of the oil to be treated, but when the amount of the extractable materials is high, it is preferable to increase the volume somewhat into the 100 to 500% range. The amount of the treating agent should be such as to form a dilute solution of the extractables for example less than 10% soap so as to avoid loss of oil in the treating solution. The

extractable materials are more soluble in and therefore more readily removable by dilute rather than more concentrated soda solutions. The treatment is accomplished at temperatures above about 350° and preferably below about 500° F. so as to avoid thermal decomposition. The more viscous the oil the higher the treating temperature will be to get a clear separation. Pressure is sufficiently high to prevent evaporation of the water from the treating solution. Residues which are solid at room temperatures may be successfully treated to remove salt, soaps, and the like.

The temperature should be kept well up within the range specified and if allowed to fall below about 350° F., there is found to be troublesome emulsification which prevents a clean separation of the aqueous from the oily layers. A small amount of oil will usually be included with the aqueous layer, which is removed while hot, but great care should be exercised to remove as completely as possible all traces of the aqueous from the oily layer. If this is carefully carried out under the conditions set forth above, no further purification of the oil is required. Water washing or cooling before separation of the water and oil layers should be avoided since this causes hydrolysis of the soda compounds of the extractable materials and causes the finished oil to have high neutralization value.

If the oil distillate is freshly obtained from crude stills while it still has a good color and is immediately subjected to the treatment with the dilute caustic alkali, no further treatment is required, but it is found that the distillate goes off color rapidly on standing and to obtain a finished oil of good color, it is often necessary to redistill the oil after the caustic treatment. The distillation is preferably carried out under vacuum in order to avoid decomposition. When treating fuel oils color and color hold are unimportant but the treatment is very effective in reducing ash content which is of great importance. Frequently when such residues are obtained by distillation over caustic soda there is enough soda present so that water may be used as the treating agent and the caustic solution is formed in situ.

The caustic treatment is capable of removing materials which cause the oil to go off in color on standing, but once these materials have developed color, the treatment is not effective in restoring color and distillation must be resorted to. The treatment may be in batch or continuous, using counterflow or parallel flow. The caustic soda may be recovered mainly by cooling to room temperature whereupon the extracted material or a large part thereof settles out and the caustic may be reused many times,

only a small amount of make up being required before it must be replaced.

As examples of the operation of the present process, the following may be considered:

**EXAMPLE 1**

A light Colombian lubricating oil distillate was heated in a closed pressure vessel with 25% of its volume of 2% aqueous caustic soda to a temperature of 400° F. A pressure of 250 pounds per square inch was maintained in the vessel so as to prevent evaporation of the caustic solution and the mixture was agitated until thorough contact was assured. The mixture was then allowed to stratify, which it did cleanly, and the aqueous liquor was drawn off while hot. The oil was redistilled under vacuum without any further treatment, giving 5.5% of light ends and 94% of a refined lubricating oil distillate.

The inspection of the original oil and the extracted and redistilled products is as follows:

|                                               | Original oil | Redis-tilled 0-70% cut | Caustic washed and redistilled 5.5-99.5% cut |
|-----------------------------------------------|--------------|------------------------|----------------------------------------------|
| Viscosity at 100° F.                          | 110          |                        | 113                                          |
| Color, Robinson                               | Dark         | 4½                     | 8½                                           |
| Color after 16 hrs. at 250° F.                |              | 2½                     | 6½                                           |
| Average lubricating oil standard <sup>1</sup> |              | 2½                     | 4+                                           |

<sup>1</sup> The average lubricating oil standard is a measure of the color stability of an average lube oil, as determined on hundreds of samples of commercial lube oils. Thus an average lube oil having an initial color of 4½ Robinson would have a color of 2½ Robinson on heating in presence of air at 250° F. for 16 hrs., and one of 8½ color would drop to 4R+ in the same test. The caustic treated oils are thus considerably better than the average oils.

|                                                                | Percent cut | Vis./100 | Color, Robinson | Color hold 16 hrs. at 250° F. | Average lube oil standard | Neut. No. |
|----------------------------------------------------------------|-------------|----------|-----------------|-------------------------------|---------------------------|-----------|
| Original oil                                                   | 100         | 342      | Black           |                               |                           |           |
| Extracted once with 78% of 0.45% caustic at 385° F., and rerun | 0-30        | 86       | 16½             | 16½                           | 11+                       | 2.23      |
|                                                                | 30-50       | 239      | 10½             | 9½                            | 9+                        | 0.05      |
|                                                                | 50-70       | 576      | 8½              | 8½                            | 4½                        | 0.08      |
|                                                                | 70-90       | 1200     | 8               | 3½                            | 4                         | 0.09      |
| Extracted once with 88% of 3.84% caustic at 385° F., and rerun | 0-30        | 84       | 17              | 13½                           | 11½                       | 0.01      |
|                                                                | 30-50       | 243      | 10½             | 9½                            | 8½                        | 0.04      |
|                                                                | 50-70       | 585      | 9½              | 6½                            | 5½                        | 0.09      |
|                                                                | 70-90       | 1235     | 8½              | 2½                            | 4                         | 0.11      |

**EXAMPLE 2**

A medium Colombian distillate having a viscosity of 274 seconds Saybolt at 100° F., was extracted with 50% of its volume of dilute caustic solution at 400° F., in the same manner described in Example 1, using a 2% caustic solution in one case and a 3% caustic solution in another case. In both cases the oil separated readily from the caustic solutions on settling at 400° F., for 5 to 10 minutes. The oils were redistilled under vacuum

without any further treatment, giving high yields of color stable lubricating oils:

|                                  | Original oil | Redis-tilled | Washed with 50% by volume of 2% aq. caustic at 400° F. and redistilled | Washed with 50% by volume of 3% aq. caustic at 400° F. and redistilled | 5  |
|----------------------------------|--------------|--------------|------------------------------------------------------------------------|------------------------------------------------------------------------|----|
| Percent cut                      | 100          | 0-98         | 0-94                                                                   | 0-97                                                                   | 10 |
| Vis./100° F.                     | 274          |              |                                                                        |                                                                        |    |
| Color, Robinson                  | Dark         | 6            | 9½                                                                     | 8½                                                                     |    |
| Color after 16 hrs. at 250° F.   |              | 1            | 7½                                                                     | 4½                                                                     |    |
| Average lubricating oil standard |              | 3+           | 5½                                                                     | 4½                                                                     |    |
| Neut. No.                        | 2.15         | 2.15         | 0.08                                                                   | 0.09                                                                   |    |
| Sap. No.                         | 2.30         | 2.30         | 0.14                                                                   | 0.28                                                                   | 15 |

By the usual acid treating method used, the yield of color stable refined oil from this stock is only about 85%, but the yield obtained by the present method averages about 10% higher for similar or better quality. 20

**EXAMPLE 3**

A total Colombian lube cut was extracted countercurrently in a tower with 78% of its volume of 0.45% aqueous caustic solution at an average tower temperature of 385° F., keeping sufficient nitrogen pressure on the system to prevent boiling of the water and in another experiment the total Colombian lube cut was extracted with 88% of its volume of 3.84% aqueous caustic solution at an average tower temperature of 385° F. Good separations of caustic extract and oil were obtained. The oils were fractionated under vacuum and separated into several cuts. The inspection of the cuts and of the untreated oil is as follows: 30 35 35

|                                                                | Percent cut | Vis./100 | Color, Robinson | Color hold 16 hrs. at 250° F. | Average lube oil standard | Neut. No. | 40 |
|----------------------------------------------------------------|-------------|----------|-----------------|-------------------------------|---------------------------|-----------|----|
| Original oil                                                   | 100         | 342      | Black           |                               |                           |           |    |
| Extracted once with 78% of 0.45% caustic at 385° F., and rerun | 0-30        | 86       | 16½             | 16½                           | 11+                       | 2.23      |    |
|                                                                | 30-50       | 239      | 10½             | 9½                            | 9+                        | 0.05      |    |
|                                                                | 50-70       | 576      | 8½              | 8½                            | 4½                        | 0.08      |    |
|                                                                | 70-90       | 1200     | 8               | 3½                            | 4                         | 0.09      |    |
| Extracted once with 88% of 3.84% caustic at 385° F., and rerun | 0-30        | 84       | 17              | 13½                           | 11½                       | 0.01      |    |
|                                                                | 30-50       | 243      | 10½             | 9½                            | 8½                        | 0.04      |    |
|                                                                | 50-70       | 585      | 9½              | 6½                            | 5½                        | 0.09      | 45 |
|                                                                | 70-90       | 1235     | 8½              | 2½                            | 4                         | 0.11      |    |

**EXAMPLE 4**

A wide cut Sugarland lube distillate having a viscosity at 100° F., of 196 seconds Saybolt was extracted twice in a countercurrent tower at an average tower temperature of 385° F., using 80% of its volume of 2% aqueous caustic solution in each treat. The original oil, and the caustic treated oil, were fractionated under vacuum and separated into 10% cuts. Inspections of these cuts were as follows: 50 55 55

|              | Percent cut | Vis./100 | Color, Robinson | Color after 16 hrs. at 250° F. | Average lube oil standard | Neut. No. | 60 |
|--------------|-------------|----------|-----------------|--------------------------------|---------------------------|-----------|----|
| Original oil | 100         | 39.2     | 1               | ¾                              | ¾                         | 0.92      |    |
|              | 0-10        | 39.2     | 21½             | 19                             |                           | 0.28      |    |
|              | 10-20       | 53.9     | 18½             | 17½                            | 13½                       | 0.52      |    |
|              | 20-30       | 77       | 17              | 11½                            | 11½                       | 0.80      |    |
|              | 30-40       | 118      | 16½             | 10½                            | 11                        | 0.95      |    |
|              | 40-50       | 196      | 13½             | 9                              | 10                        | 0.98      |    |
|              | 50-60       | 338      | 11              | 8½                             | 9½                        | 0.95      |    |
|              | 60-70       | 617      | 10½             | 5                              | 8½                        | 0.92      |    |
|              | 70-80       | 1120     | 9               | 4½                             | 4½                        | 0.88      |    |
|              | 80-90       | 1688     | 8½              | 3                              | 4½                        | 0.86      |    |
|              | 90-100      | 39.8     | 21½             | 18½                            |                           | 0.03      |    |
|              | 10-20       | 55.0     | 18½             | 17½                            | 12½+                      | 0.03      |    |
|              | 20-30       | 78.4     | 17              | 14½                            | 11½                       | 0.05      | 70 |
|              | 30-40       | 125      | 16½             | 12                             | 11+                       | 0.05      |    |
|              | 40-50       | 210      | 14½             | 10                             | 10½                       | 0.06      |    |
|              | 50-60       | 340      | 12½             | 9½                             | 9½                        | 0.06      |    |
|              | 60-70       | 600      | 10½             | 9                              | 9+                        | 0.08      |    |
|              | 70-80       | 1080     | 9½              | 6                              | 5½                        | 0.11      |    |
|              | 80-90       | 1627     | 8½              | 4½                             | 4½                        | 0.14      |    |

In this case even the cuts from the untreated oil were fairly color stable especially the light viscosity ones, but caustic treating improved the color stability considerably. The treatment was particularly effective with the 1000 to 1600 viscosity cuts (70-80% and 89-90%) which were color stable while the untreated ones were not.

## EXAMPLE 5

10 A light Colombian lube distillate was treated with 15 pounds of 91% sulfuric acid at about 90° F. On settling, the sludge was drawn off and the oil was neutralized with caustic. The neutral oil so obtained which contained about 0.02% ex-

15

| Cut No.                        | Oil treated with recovered caustic and redistilled |                 |                 |                 |                                                           |                  |                 |                 | Oil treated with fresh caustic one 50% countercurrent treat at 380 to 390° F. |                  |                 |                 |
|--------------------------------|----------------------------------------------------|-----------------|-----------------|-----------------|-----------------------------------------------------------|------------------|-----------------|-----------------|-------------------------------------------------------------------------------|------------------|-----------------|-----------------|
|                                | One 35% countercurrent treat at 380-390° F.        |                 |                 |                 | Two counter current treats at 380-390° F. (38+25% treats) |                  |                 |                 | Oil treated with fresh caustic one 50% countercurrent treat at 380 to 390° F. |                  |                 |                 |
|                                | 1                                                  | 2               | 3               | 4               | 1                                                         | 2                | 3               | 4               | 1                                                                             | 2                | 3               | 4               |
| Vis./100                       | 75.7                                               | 213             | 545             | 1301            | 79.1                                                      | 221              | 555             | 1318            | 77                                                                            | 220              | 531             | 1298            |
| Color, Robinson                | 16 $\frac{1}{2}$                                   | 11              | 9               | 7               | 16 $\frac{1}{2}$                                          | 10 $\frac{1}{2}$ | 9               | 7 $\frac{1}{2}$ | 16 $\frac{1}{2}$                                                              | 11 $\frac{1}{2}$ | 9               | 7 $\frac{1}{2}$ |
| Color after 16 hrs. at 250° F. | 11                                                 | 9 $\frac{1}{2}$ | 4 $\frac{1}{2}$ | 2 $\frac{1}{2}$ | 12 $\frac{1}{2}$                                          | 9                | 5 $\frac{1}{2}$ | 2 $\frac{1}{2}$ | 16 $\frac{1}{2}$                                                              | 9 $\frac{1}{2}$  | 5               | 1 $\frac{1}{2}$ |
| Average lube oil standard      | 11 $\frac{1}{2}$                                   | 9 $\frac{1}{2}$ | 4 $\frac{1}{2}$ | 3 $\frac{1}{2}$ | 11 $\frac{1}{2}$                                          | 9                | 4 $\frac{1}{2}$ | 3 $\frac{1}{2}$ | 11 $\frac{1}{2}$                                                              | 9 $\frac{1}{2}$  | 4 $\frac{1}{2}$ | 3 $\frac{1}{2}$ |
| Neut. No.                      | .05                                                | .06             | .09             | .12             | .03                                                       | .03              | .05             | .08             | .05                                                                           | .05              | .08             | .11             |

cess caustic was distilled under vacuum in a refinery pipe still, and another sample of the same oil was washed twice in a bomb with 25% of its volume of 2% caustic each time, at 400° F., and still another sample was washed twice with 50% of its volume of water each time at 460° F. Both the samples of washed oils were vacuum distilled in a laboratory still. Ash contents of the oils before distillation were as follows:

| Per cent ash                                                    |       |
|-----------------------------------------------------------------|-------|
| 40 Acid treated and neutralized oil                             | 0.65  |
| Acid treated and neutralized oil washed with caustic at 400° F. | 0.008 |
| Acid treated and neutralized oil washed with water at 460° F.   | 0.04  |

Inspection of the distillates obtained from these oils was as follows:

## Acid treated and neutralized light Colombian distillate

| 55                             | Fractionated in refinery pipe still | Washed with 2% caustic at 400° F. (2x25% treats) and fractionated in the laboratory |                 |                  |                  | Washed with water at 460° F. (2x50% treats) and fractionated in the laboratory |                 |                  |                  | 55              |                 |     |
|--------------------------------|-------------------------------------|-------------------------------------------------------------------------------------|-----------------|------------------|------------------|--------------------------------------------------------------------------------|-----------------|------------------|------------------|-----------------|-----------------|-----|
|                                |                                     | Vis./100                                                                            | 240             | 908              | 71.2             | 211                                                                            | 344             | 903              | 76.5             | 236             | 514             | 997 |
| Vis./100                       | 72.3                                | 240                                                                                 | 908             | 71.2             | 211              | 344                                                                            | 903             | 76.5             | 236              | 514             | 997             |     |
| Color, Robinson                | 17 $\frac{1}{2}$                    | 11 $\frac{1}{2}$                                                                    | 8 $\frac{1}{2}$ | 17 $\frac{1}{2}$ | 14 $\frac{1}{2}$ | 11 $\frac{1}{2}$                                                               | 8 $\frac{1}{2}$ | 17               | 12 $\frac{1}{2}$ | 9 $\frac{1}{2}$ | 6 $\frac{1}{2}$ |     |
| Color after 16 hrs. at 250° F. | 4 $\frac{1}{2}$                     | 3                                                                                   | 2 $\frac{1}{2}$ | 16 $\frac{1}{2}$ | 10 $\frac{1}{2}$ | 9 $\frac{1}{2}$                                                                | 4 $\frac{1}{2}$ | 16 $\frac{1}{2}$ | 10 $\frac{1}{2}$ | 8 $\frac{1}{2}$ | 2 $\frac{1}{2}$ |     |
| Average lube oil standard      | 11 $\frac{1}{2}$                    | 9 $\frac{1}{2}$                                                                     | 4 $\frac{1}{2}$ | 11 $\frac{1}{2}$ | 10 $\frac{1}{2}$ | 9 $\frac{1}{2}$                                                                | 4 $\frac{1}{2}$ | 11 $\frac{1}{2}$ | 9 $\frac{1}{2}$  | 5 $\frac{1}{2}$ | 3 $\frac{1}{2}$ |     |
| Neut. No.                      | 0.04                                | 0.05                                                                                | 0.06            | 0.04             | 0.04             | 0.07                                                                           | 0.08            | 0.68             | 1.46             | -----           | 1.16            | 60  |

It will be noted that on washing with water at 460° F., the neutralization values of the distillates were very high, showing that the soaps had been hydrolyzed to a large extent, whereas the very low ash content (0.008%) of the caustic washed oil and the low neutralization values of the distillates show that the soap was washed out thoroughly with 2% caustic solution at 400° F.

70

## EXAMPLE 6

When using large volumes of caustic solution for extractions of acids and unstable compounds from petroleum oils, it is necessary to recover the excess caustic. This is easily done, since on

cooling the caustic extracts to room temperature or lower, practically all the extracted material separates out of solution, leaving a recovered caustic which may be used over again. In order to prove that the recovered caustic is just as effective for extraction of lube distillates as fresh caustic of corresponding strength, the total Colombian lube cut mentioned in Example 3 was extracted countercurrently at 380 to 390° F., (1) with recovered caustic containing 1.76% free NaOH and (2) with fresh caustic containing 2% NaOH. The extracted oils were vacuum fractionated and inspections of the distillates were as follows:

5

10

15

20

25

30

35

40

45

65

70

75

## EXAMPLE 7

A sample of pipe still bottoms obtained on stripping off the lubricating oil distillates from an acid treated and neutralized Colombian distillate in a refinery pipe still was washed with dilute caustic at 470° F. Analysis of the original pipe still bottoms showed that it had approximately the following composition:

|                       | Per cent |
|-----------------------|----------|
| Heavy oil             | 50       |
| Inorganic salts       | 6        |
| Soaps (by difference) | 44       |

and the ash content was 12.89%

On washing these bottoms with 300% of its volume of 0.5% caustic at 470° F. by mixing thoroughly in a closed bomb under equilibrium pressure for 30 minutes, followed by settling for 5 minutes, a clear separation of oil and extract was obtained. 42 volumes of oil were recovered from

each 100 volumes of bottoms charged to the bomb, indicating that 84% of the oil was recovered. This oil had a gravity (A. P. I.) of 17.0 and a viscosity at 210° F., of 263 seconds Saybolt—and is suitable as such for lubrication of heavy machinery or for grease manufacture or the like; if desired the oil may be redistilled for production of heavy cylinder oil. The extract from the soap bottoms was acidified with sulfuric acid, and the organic acids so liberated were washed with water at 200° F. On vacuum distillation of these acids, 60% of them distilled over at bottoms temperatures ranging from 400° F. to 600° F., under 5 mm. Hg pressure. The distillate

had a color of 8 Robinson and had the characteristic odor of crude naphthenic acids. Inspection of this distillate was as follows:

Color ----- 8R  
5 Neut. No ----- 123.5  
Sap. No ----- 123.5

These acids may be further purified in various ways, but substantially oilfree acids may be obtained by the method described above by increasing the amount of dilute caustic used for the extraction of the soaps from the pipe still bottoms, since the oil is relatively much less soluble in dilute soap solutions than in concentrated ones.

15 The present invention is not to be limited to any theory of the chemical reactions involved in the treatment nor to any particular alkali.

I claim:

1. An improved method for refining heavy hydrocarbon oils by extraction comprising treating the oil with dilute aqueous caustic soda of up to 5% concentration under pressure high enough to maintain the hydrocarbon oil and caustic solution liquid at the operating temperature, which is above 300° F., and below the decomposing temperature of the hydrocarbon oil, and removing the dilute caustic soda solution and ex-

tracted material from the oil while hot by decantation.

2. An improved process according to claim 1 in which the treating solution is an aqueous solution containing .25 and 5% of caustic soda.

3. Process according to claim 1 in which the dilute caustic soda is recovered for reuse by cooling and separating the extracted material.

4. An improved process for refining lubricating oil from naphthenic crudes which are susceptible to serious loss of color on standing, consisting of the steps of bringing the oil into contact with an aqueous caustic soda solution of from .25 to about 5% while at a temperature between 350 and 500° F., under pressure sufficient to maintain the oil and caustic solution in liquid phase and separating the treating agent from the refined oil while hot by decantation.

5. An improved process according to claim 4 in which the treatment is effected continuously by treating a flowing stream of the oil with caustic soda solution.

6. Process according to claim 4 in which the treatment is effected by treating a flowing stream of oil countercurrently with a stream of the caustic solution.

HANS G. VESTERDAL.